

## UNITED STATES PATENT OFFICE

2,138,797

## MANUFACTURE OF IRON

Marvin J. Udy, Niagara Falls, N. Y., assignor to  
Monsanto Chemical Company, a corporation  
of Delaware

No Drawing. Original application December 3,  
1934, Serial No. 755,767. Divided and this ap-  
plication August 7, 1937, Serial No. 157,840

3 Claims. (Cl. 75—123)

This application is a division of Serial No.  
755,767 filed Dec. 3, 1934.

This invention relates to the manufacture of  
iron, steel and alloys thereof, and has for its  
5 principal object the provision of a process for  
the economic production thereof.

A further object of this invention is the pro-  
vision of a process for the production of iron of a  
high degree of purity.

10 A still further object of this invention is the  
recovery of phosphatic values in the metallurgy  
of iron.

In previously known related processes it is the  
practice to treat a phosphatic pig iron, to which  
15 may have been added scrap iron, with lime and  
iron ore or mill scale until the impurities have  
been decreased to the desired degree. In a modi-  
fication of the basic open-hearth process, known  
as the Hoesch Process (Bradley Stoughton—

20 Metallurgy of Iron and Steel—1913, page 149)  
wherein a highly phosphatic slag is recovered,  
this process results in the production of steel.  
This process utilizes a relatively low slag volume  
25 and results, during the first part thereof, in the  
removal of 55% of the carbon, 86% of the phos-  
phorus, 64.6% of the manganese, and 38% of the  
sulfur, together with all of the silicon. From  
30 these results it is evident that sulfur is removed  
with great difficulty and that the removal of the  
remaining impurities, with the exception of  
silicon, is also attended with some degree of dif-  
ficulty.

I have now discovered that the manufacture  
of iron and/or steel may be considerably simpli-  
35 fied and a purer product obtained if, instead of  
selecting a raw material with a low content of  
impurities, I deliberately choose or prepare an  
alloy of high, or relatively high, impurity content  
40 and then remove the impurities in the alloy by  
means of the proper slag. My discovery is based  
upon the observation that when such alloys as  
ferrophosphorus, ferrosilicon or ferromanganese,  
which normally contain a relatively high propor-  
45 tion of the alloying constituents, are treated with  
a basic oxidizing slag, not only are those ele-  
ments which are present in major proportions ef-  
fectively removed but the ordinary impurities  
which are present in minor proportions, such as  
50 sulfur, tin, and others, are also removed and more  
effectively than has hitherto been observed.

For the purpose of the present specification and  
claims I shall confine myself to ferrous alloys,  
such alloys having, in addition to the iron neces-  
sarily present, alloying elements such as phos-  
55 phorus, silicon and manganese, which elements  
are present in major proportions, that is, in  
amount, say, about 10% by weight of the alloys.  
I am not necessarily confined to the use of a  
single alloying element combined with iron in  
60 the ferrous alloy, but may employ an alloy con-

taining two or more alloying elements combined  
with iron. Examples of suitable alloys are ferro-  
phosphorus-silicon, ferromanganese-phosphide,  
ferromanganese-silicon. In the case where two  
or more alloying elements combined with iron  
are employed, I prefer to have the sum of such  
5 alloying elements other than iron total at least  
10 per cent of the weight of the alloy, although  
such requirement is subject to some degree of  
flexibility, as will later more fully appear.

In addition to the alloying constituents pres-  
ent in major proportion, most ferrous alloys con-  
tain varying amounts of elements which may be  
termed impurities. These elements may consist  
of sulfur, titanium, vanadium, chromium, tin, etc. 15  
Another source of the minor impurities entering  
my process will consist in the use of scrap iron,  
the application of which will presently more fully  
appear.

A further variation of my process is exemplified 20  
by the production of pure or ingot iron. As is  
well known in the production of pure iron, it has  
been customary to use pig iron or scrap with as  
low a content of impurities as possible, and then  
to treat the molten bath with suitable eliminating  
25 agents to combine with the impurities present.  
Such treatment was necessarily carried out in a  
high powdered open-hearth furnace and involved  
a long-time treatment at a high temperature.  
The production of pure or ingot iron by these 30  
prior processes involved the careful selection of  
the raw materials; for example, it was customary  
to select, as a starting material, a pig iron of  
the following analysis:

Phosphorus—not over 1.00 and as low as pos- 35  
sible.

Sulfur—not over 0.05 and as low as possible.

Silicon—not over 2.00 and as low as possible.

Instead of employing materials of a high de-  
gree of purity, that is a high iron content, I 40  
make use of ferro-alloys having a comparatively  
low iron content and treat such alloys in the  
molten state with a basic oxidizing slag whereby  
the major alloying elements, together with the  
impurities present therein, and those added by 45  
the addition agents, are substantially eliminated.  
By this means I may obtain a pure or ingot iron  
in which the ordinary impurities may be within  
the following ranges in percentages:

|            |   |       |    |       |
|------------|---|-------|----|-------|
| Phosphorus | — | 0.10  | to | 0.001 |
| Silicon    | — | 0.10  | to | 0.004 |
| Carbon     | — | 0.14  | to | 0.01  |
| Sulfur     | — | 0.003 | to | 0.001 |

Such an ingot iron is quite comparable with  
and in some cases may exceed the purity of in-  
got iron produced by earlier known processes.

As in earlier known processes, the selection of  
the materials to be treated by my process is of  
some importance, though the purity of the raw

materials, as regards metalloids other than the major alloying element, is not so important as in the earlier known processes for the reason that I make use of more powerful scavenging forces than were hitherto known. Regarding the content of the major alloying element, it may be said, as a general principle, that I desire such element to be as high as practical, the actual percentage being usually dictated by economic considerations. This upper limitation is suggested by my observation that the scavenging effect on metalloids or minor impurities which are usually difficult to remove will be a maximum. It is also my observation that the amount of the major alloying element present in the metallic raw material may be graduated to suit the amount of minor non-metallic raw materials to be removed during the refining operation. In general it may be said that the greater the amount of the major alloying element scavenged from the molten alloy, the greater will be the elimination of the associated minor impurities.

As a practical example of my process, I will describe its operation with respect to the treatment of ferrophosphorus, this being an alloy of iron and phosphorus of commercial importance at the present time.

For practical purposes I prefer to use, as starting material, a commercial grade of ferrophosphorus, such, for example, as may be prepared by smelting phosphatic and iron-bearing materials either in the blast or electric furnace. Such materials usually have a phosphorus content varying from 15% to 28% and, as such, are directly useable in my process. In many cases, however, I may add to such commercial iron-phosphorus alloys an additional amount of iron either as cast iron or scrap, being careful, however, that the total phosphorus content of the mixture is not lowered appreciably below 10%. For the purpose of the present specification and claims, I shall designate such an alloy as an iron containing a relatively high proportion of phosphorus, since, as may be seen from the prior art, the phosphorus content is much greater than that hitherto considered practicable.

Accordingly, I produce first an iron-phosphorus alloy or ferrophosphorus either by smelting scrap iron and phosphatic material in an electric furnace according to the method taught by Carotherers in U. S. Patent 1,410,550, or that described by Gray in U. S. Patent 831,427. The source of iron in the former case may be any suitable scrap material or it may be an ore of iron. In the latter process ore is usually employed. The ferrophosphorus produced in the electric furnace will vary in content from 17% to 28% phosphorus, and from 0.1% to 3.0% silicon; while that produced in the blast furnace will average 16% to 21% phosphorus, 0.1% to 1.0% silicon, and 0.1% to 1.0% sulfur.

I next provide a basic lined furnace, either a gas-fired, open-hearth or an electric type being suitable, and, if conveniently located to the ferrophosphorus furnace, I may charge the basic furnace directly with molten ferrophosphorus. Before charging the furnace with the molten ferrophosphorus, it is desirable to provide a basic oxidizing slag, which is done by charging to the furnace a mixture of lime and iron ore. The proportions used will usually approximate 14 pounds of lime to 20 pounds of iron ore containing, say 76%  $Fe_2O_3$ , although these proportions may be varied to suit the requirements of the refining operation and of the slag produced. The molten

ferrophosphorus is then run into the furnace at a controlled rate so that the reaction does not become too violent.

A rapid elimination of the phosphorus now takes place with considerable evolution of heat in the bath. When the phosphorus in the metal has decreased to from 1 to 3 per cent, the slag is removed and replaced with a fresh slag of the same character as first used. The refining operation is continued at a high heat until the phosphorus in the metal has been reduced to between 0.10% and 0.001%. At this point the metal is withdrawn into a ladle, and degasifying or deoxidizing agents are added. These may consist of aluminum or ferrotitanium in relatively small amounts. The molten alloy is now cast into ingot molds.

In certain cases I may employ the ferrophosphorus in lump form, by adding such material directly to the basic oxidizing slag. By proper choice of lump size the vigor of the reaction may be controlled. During the addition of the ferrophosphorus lumps or before such addition, I may add additional quantities of iron as cast or scrap iron.

Because of the rapidity with which the charge can be heated in the electric furnace, some advantage will result from operating in this type of furnace. There will be a greater contamination with carbon when operating in such a furnace; however, for certain purposes this may not be objectionable.

The amount of basic oxidizing slag used in the first refining is proportioned so that it will contain from 18 to 24% of phosphoric acid as  $P_2O_5$  when finished, although this figure will vary somewhat.

In prior processes for the production of steel and iron the amount of slag formed amounted to from 10% to 30% by weight of the amount of such iron or steel treated. My process, on the other hand, consists in the treatment of iron alloys with from 100% to 400% by weight of slag based on the amount of iron produced.

An examination of the metal from under the first slag produced as described above shows that the metalloids, other than phosphorus, have been substantially removed from the iron.

The amount of basic oxidizing slag used in the second refining operation may be equal in amount to that first used. Because of the lower phosphorus in the metal, however, such slag will contain less phosphoric acid. The removal of the refined metal from below this second slag is conveniently done by pouring it from below, as is done in a tilting furnace. The second slag will then remain in the furnace and, being of low phosphorus content, may be used as a first refining slag in a subsequent operation. Additional quantities of slagging ingredients may be added, if desired.

The impurities present in the iron produced according to my process will be within the following ranges:

|            |                |    |
|------------|----------------|----|
| Phosphorus | 0.10 to 0.001  | 65 |
| Silicon    | 0.10 to 0.004  |    |
| Carbon     | 0.14 to 0.01   |    |
| Sulfur     | 0.003 to 0.001 |    |

The actual amount of impurity present in the iron produced by my process will be dependent upon the type of furnace used and the care taken in operating the same. In general, a slightly higher carbon content will be obtained in the electric furnace than in the open-hearth furnace. 75

The pure iron produced will analyze between 99.56 and 99.98% Fe, and is especially suited for uses where a high degree of corrosion resistance is desired. Because of its freedom from the 5 usual impurities, it is also favored for the manufacture of special iron alloys or steel.

The intermediate product produced under the first refining slag may contain from 0.6 up to 2 or 3 per cent of phosphorus. If the phosphorous is to be further reduced by subsequent 10 treatment, it is advantageous to stop the treatment with the first slag when the phosphorus in the metal is in the neighborhood of 2 or 3 per cent. If, however, a high phosphorus ingot iron 15 is desired, it is best to carry the scavenging of the phosphorus down with the first slag until the content of this element is in the range of from 0.65 to about 1.07% phosphorus. When carried to this point, the minor impurities present, namely, 20 the carbon, manganese, silicon and sulfur, will total in the aggregate less than 0.30% and usually somewhat more than 0.015% of the alloy.

The high phosphorous iron may be cast into ingots, forged and rolled or otherwise fabricated. 25 When hot rolled and annealed, a 22-gauge iron sheet prepared from an ingot iron containing between 0.65% and 1.07% phosphorus will have an ultimate tensile strength of from 80,000 to 85,500 pounds per square inch, a yield point of 70,000 30 to 73,000 pounds per square inch, and an elongation in 2 inches of from 15% to 20%.

While I am uncertain as to the exact reason for the almost complete elimination of the impurities in the metal produced by my process, I believe it to be connected with the elimination of the large amount of the major alloying element such, for example, as phosphorus present in proportion to the iron. Apparently the scavenging 35 of the large quantities of phosphorus which I employ carries into the slag most of the impurities present in the iron and iron ore.

This scavenging action is particularly noticeable in the case of sulfur, which may be present in the original raw materials in rather large 45 quantities. I have found, for example, in one case that where sulfur was present in the ferro-phosphorus alloy to the extent of 0.65%, one treatment with a basic oxidizing slag served to reduce the amount of this impurity to 0.03%. This corresponds to a sulfur elimination of 96%.

The scavenging action of the phosphorus present in the high phosphorus-iron alloy is, of course, not confined to its effect on sulfur, but is also effective in removing silicon, manganese, tin, etc. As I have indicated above, the metal resulting 50 from my process is characterized by a

very low content of those impurities normally present in commercial iron or steels, and is thereby distinguished over the prior art products and process.

My process is effective, as has already been 5 stated, not only with ferrophosphorus but also with ferrosilicon, ferromanganese and mixtures of these alloys. For most practical results I prefer to limit the content of the major allowing elements to between 10% on the lower side to as 10 high as 28% on the upper side, the remaining element being essentially iron. When working within these limits, which, as has already been 15 stated, may be varied depending upon conditions, I have found that removal of the minor impurities occurring in ferro alloys becomes a comparatively simple process.

Having obtained a purified iron by the above-described process, I may produce therefrom either carbon steel or any of the various alloy steels by 20 the addition of the proper alloying constituents.

In the foregoing specification I have described 25 various specific means by which my process may be carried out. It will be apparent, however, to those skilled in the art that my invention is susceptible to various changes and modifications without departing from the spirit thereof; and I desire, therefore, that my invention be not limited to any specific modifications except as indicated by the prior art or as specifically set 30 out in the appended claims.

What I claim is:

1. An ingot iron containing:

|            | Per cent               |    |
|------------|------------------------|----|
| Phosphorus | between 0.60 and 3.00  | 35 |
| Silicon    | between 0.10 and 0.004 |    |
| Carbon     | between 0.14 and 0.01  |    |

the remainder being iron.

2. An ingot iron containing:

|             | Per cent                |    |
|-------------|-------------------------|----|
| Phosphorous | between 0.65 and 1.07   | 40 |
| Silicon     | between 0.10 and 0.004  |    |
| Carbon      | between 0.14 and 0.01   |    |
| Sulfur      | between 0.003 and 0.001 |    |

the remainder being iron.

3. An ingot iron containing:

|             | Per cent                |    |
|-------------|-------------------------|----|
| Phosphorous | between 0.65 and 1.07   |    |
| Silicon     | between 0.10 and 0.004  |    |
| Carbon      | between 0.14 and 0.01   | 50 |
| Sulfur      | between 0.003 and 0.001 |    |

the remainder being iron, said ingot iron having a tensile strength of more than 80,000 pounds per square inch.

MARVIN J. UDY.